

# United States Patent Office

3,043,683

Patented July 10, 1962

1

3,643,683

NIOBIUM-TITANIUM CHROMIUM ALLOY  
Hugh B. Hix, Wilmington, Del., assignor to E. I. du Pont de Nemours and Company, Wilmington, Del., a corporation of Delaware  
No Drawing. Filed Sept. 23, 1959, Ser. No. 841,683  
7 Claims. (Cl. 75—174)

This invention pertains to novel niobium base alloys, and more particularly to outstanding high temperature strength and oxidation resistant, ternary alloys containing niobium, titanium, and chromium.

In present-day industry there is an ever-increasing need for metals which are utilizable at very high temperatures. This need has taken on considerable importance as a result of developments in jet engine aircraft and the field of atomic power. In addition to these important uses, high temperature metals are also employed in gas turbines of all types, dies for high temperature working of metals, high temperature reactors, and the like. For a metal to be suitable as a material of construction in high temperature equipment, it must possess, in addition to a high melting point, strength and oxidation resistance at the operating temperatures of the equipment. Furthermore, the metal must be ductile in order to permit its fabrication. It is, therefore, an object of this invention to provide improved, workable alloys which possess unusually high oxidation resistance and strength at elevated temperatures. It is a further object to provide a metal alloy suitable as a material of construction in high temperature equipment of all types.

It has now been found that workable alloys possessing unusually high corrosion resistance and strength at high temperatures can be produced by alloying titanium, chromium, niobium, and the specified optional elements in the amounts set forth herein. It is, therefore, an object of this invention to provide improved, workable alloys which possess unusually high oxidation resistance and strength at elevated temperatures. It is a further object to provide an alloy suitable as a material of construction in high temperature equipment of all types.

The alloys of this invention comprise niobium base compositions containing about 5-30% by weight of titanium, about 1-30% by weight of chromium, and the balance being essentially niobium in an amount of at least 50% by weight.

In addition to the above-named essential elements, the alloy may contain about 0-7% of aluminum, about 0-2% carbon, about 0-2% cobalt, about 0-7% iron, about 0-7% manganese, about 0-2% nickel, about 0-2% silicon, about 0-7% tantalum, about 0-7% tungsten, about 0-7% vanadium, about 0-7% zirconium, the sum total of the added elements Al, C, Co, Fe, Mn, Ni, Si, Ta, W, V, and Zr ranging from about 0-7% by weight. In a more preferred embodiment, the above constituents are in the amounts stated except that the sum total of the optional elements Al, C, Co, Fe, Mn, Ni, Si, Ta, W, V, and Zr ranges from about 2-5%.

In another preferred embodiment, the alloys of this invention comprise about 10-25% titanium, about 15-30% chromium, and the balance being essentially niobium in an amount of at least 50% by weight. In addition, the alloy of this preferred embodiment may contain about 0-5% of aluminum, about 0-2% carbon, about 0-2% cobalt, about 0-5% iron, about 0-5% manganese, about 0-2% nickel, about 0-2% silicon, about 0-5% tantalum, about 0-5% tungsten, about 0-5% vanadium, about 0-5% zirconium, the sum total of the added elements Al, C, Co, Fe, Mn, Ni, Si, Ta, W, V, and Zr ranging from about 0-5% by weight.

In a more preferred embodiment, the alloys of this invention comprise about 15-25% titanium, about 20-

2

28% chromium, and the balance being essentially niobium in an amount of at least 50% by weight. In addition, the alloy of this embodiment may contain about 0-5% of aluminum, about 0-2% carbon, about 0-2% cobalt, about 0-5% iron, about 0-5% manganese, about 0-2% nickel, about 0-2% silicon, about 0-5% tantalum, about 0-5% tungsten, about 0-5% vanadium, about 0-5% zirconium, the sum total of the added elements Al, C, Co, Fe, Mn, Ni, Si, Ta, W, V, and Zr ranging from about 0-5% by weight, the balance being niobium in an amount in excess of 50% by weight.

The alloys of this invention may be prepared by conventional metal melting and remelting techniques using inert conditions. The individual metals are melted together, solidified and remelted until homogeneity is obtained. The final melt is then allowed to cool and solidify into a desired shape. The case material thus obtained is of a workable metal with strength and oxidation resistance at high temperatures, and it is suitable as a material of construction in high temperature equipment designed to operate at temperatures beyond the limits of present equipment constructed of the best high temperature alloys.

These new alloys may be prepared in any of a number of types of melting furnaces. The one used in the working examples, which follow, was an arc melting furnace of the type described by W. Kroll in "Transactions of the Electrochemical Society," vol. 78, pp. 35-47, 1940. This furnace has an integral, water-cooled copper crucible in which the charge may be melted and solidified. The charge of metal constituents for this furnace may be in any convenient form; e.g., powder, shot, wire, sponge, etc. Another suitable melting apparatus is a compressed, consumable arc electrode furnace as described in U.S. Patent 2,640,860 to S. A. Herres. Also, one may use a combination of non-consumable and consumable electrodes in a double melt furnace such as is described in U.S. Patent 2,541,764 to the above-mentioned Mr. Herres. A continuous feed furnace such as is described in U.S.P.B. Report 111,083 may also be used. Furthermore, melting could be accomplished by inductively heating the charge in a suitable crucible. Regardless of the melting apparatus used, care should be exercised to protect the molten metals from the normal atmosphere since contamination of the alloy by oxygen, nitrogen, etc. is to be avoided. To prevent this contamination the melting should be carried out under inert conditions, such as an atmosphere of argon or a protective slag or a combination of a protective slag and a controlled atmosphere. The practice of using an inert atmosphere when melting metals is well known in the art.

The following examples are presented to illustrate the preparation of specific alloys of this invention and the outstanding properties of these alloys. These examples are illustrative only and are not to be construed as limiting the invention. All percents set forth in the ensuing examples refer to percents by weight.

## EXAMPLE I

An alloy of the following composition was prepared: 15 titanium, 23% chromium, 59% niobium, 1% tungsten, and 2% tantalum. The procedure for preparing this alloy was as follows: The individual metal constituents were melted together in a furnace having an integral, water-cooled copper crucible, as described by Kroll in the "Transactions of the Electrochemical Society" publication referred to above. A helium atmosphere was maintained, and the alloy composition was alternately remelted and solidified six times, whereupon a homogeneous ingot was obtained.

Table I below sets forth the oxidation resistance possessed by the alloy of this example. Oxidation resistance is determined by the following procedure: Weighed sam-

ples of the alloy (in a porcelain crucible which was slotted to insure adequate access of air to the ingot) were placed in a resistance furnace wherein the resistors are silicon carbide rods and exposed for at least 16 hours at 1000° C. to an air purge of 2 cu. ft./min. After exposure, the samples were cooled and weighed, and the amount of oxidation was determined as the percent weight gain in the sample.

Table I

|                    | Percent weight gain | 10 |
|--------------------|---------------------|----|
| Alloy of Example I | 1.5                 |    |
| Unalloyed niobium  | 20                  |    |

The Rockwell hardness of the alloy was 48.

The ultimate strength for the alloy of Example I is given below and for purposes of comparison data on good, commercially available alloys are also given:

|                                                                                                      |                                 | P.s.i.   |    |
|------------------------------------------------------------------------------------------------------|---------------------------------|----------|----|
| Alloy of Example I                                                                                   | Ultimate strength at room temp. | >200,000 |    |
| Commercial Alloy B: 80% Ni, 20% Cr.                                                                  | Ultimate strength at 1,150° C.  | >100,000 |    |
| Commercial Alloy C: 38% Co, 28% Ni, 20% Cr, 7% W, 4% Ti, 2% Fe, 0.2% C.                              | Ultimate strength at room temp. | 163,000  |    |
| Commercial Alloy D: 42% Co, 20.5% Ni, 20% Cr, 4.2% W, 4% Nb, 4% Mo, 3% Fe, 1.3% Mn, 0.6% Si, 0.4% C. | Ultimate strength at 870° C.    | 42,000   |    |
|                                                                                                      | Ultimate strength at 982° C.    | 20,000   |    |
|                                                                                                      | Ultimate strength at room temp. | 150,000  | 25 |
|                                                                                                      | Ultimate strength at 871° C.    | 50,000   |    |

## EXAMPLE II

An alloy of the following composition was prepared according to Example I: 22% titanium, 24% chromium, 51% niobium, 1% cobalt, 0.3% silicon, 1.7% tantalum.

In the oxidation test described in Example I this alloy will show a 0.9% weight gain, as compared with 20% weight gain for unalloyed niobium. The Rockwell hardness is 49. The alloy exhibits an ultimate strength of >200,000 p.s.i. at room temperature and >100,000 p.s.i. at 1150° C.

## EXAMPLE III

Using the procedure of Example I and a charge consisting of 11.2% titanium, 19.2% chromium, and 69.6% niobium, an alloy was made and tested for ultimate strength at room and elevated temperatures. The following data are the results of the tests and a comparison of such data with good, commercially available alloys:

Table II

|                          | Alloy Composition                                                                | Temperature          | Ultimate Strength, p.s.i. |  |
|--------------------------|----------------------------------------------------------------------------------|----------------------|---------------------------|--|
| Alloy A (this invention) | 69.6% Nb, 19.2% Cr, 11.2% Ti                                                     | room temp. 1,300° C. | 240,000 108,000           |  |
| Alloy B                  | 80% Ni, 20% Cr.                                                                  | room temp. 871° C.   | 163,000 42,000            |  |
| Alloy C                  | 38% Co, 28% Ni, 20% Cr, 7% W, 4% Ti, 2% Fe, 0.2% C.                              | 982° C.              | 20,000                    |  |
| Alloy D                  | 42% Co, 20.5% Ni, 20% Cr, 4.2% W, 4% Nb, 4% Mo, 3% Fe, 1.3% Mn, 0.6% Si, 0.4% C. | room temp. 871° C.   | 150,000 50,000            |  |

The room temperature yield strength of applicant's Alloy A at 0.2% offset is 180,000 p.s.i., thus showing this alloy has useful ductility at room temperature. Advantaneously, it also appears to exhibit a recrystallization temperature in excess of 1300° C.

In order to show how the alloys of this invention compare with a standard commercial alloy at the same elevated temperature, Alloys A and C of Table II were formed into 1/2" cubes and subjected to compressive stress at 1200° C. and 1300° C. Table III shows the results of these tests at 1200° C.

4  
Table III

|   | Pressure Applied in Pounds/Sq. In. at 1,200° C. (2,192° F.) | Alloy C                                                                                      | Alloy A (this invention)      |
|---|-------------------------------------------------------------|----------------------------------------------------------------------------------------------|-------------------------------|
| 5 | 100,000 p.s.i. >300,000 p.s.i.                              | deforms 50% in 30 sec. no test undertaken in view of obvious failure under these conditions. | no flow. 50% upset in 30 sec. |

The above Table III shows that Alloy C deformed very rapidly at 1200° C. under a pressure of 100,000 p.s.i., whereas Alloy A did not flow. It will be seen that at a pressure >300,000 pounds per sq. in. a 50% upset could be obtained with no indication of edge cracking. The fact that this alloy did upset at a pressure above 300,000 p.s.i. without edge cracking is important since it shows that the material is non-brittle and capable of being worked when sufficient force is used, thus making the alloy suitable for fabrication into high temperature equipment.

Table IV shows a comparison of results when Alloys A and C were subjected to stress at 1300° C.

Table IV

|    | Pressure Applied in Pounds/Sq. In. at 1,300° C. (2,372° F.) | Alloy C                                            | Alloy A (this invention)                             |
|----|-------------------------------------------------------------|----------------------------------------------------|------------------------------------------------------|
| 30 | 100,000 p.s.i.                                              | sample crumbled before maximum stress was applied. |                                                      |
| 35 | 110,000 p.s.i.                                              |                                                    | anvils crumbled but there was no upset in the alloy. |

Alloy A in the "as cast" state was subjected to a force in excess of 300,000 lbs./sq. in. at 1200° C. as reported in Table III. Examination of the microstructure of Alloy A at 250 magnification before it was subjected to the above force showed that it was composed of two phases, the lighter phase being a continuous phase. A scratch test made upon the metal by means of a diamond indenter drawn across the surface under constant load did not scratch the continuous phase, showing that this is the harder phase. The discontinuous phase was, however, scratched, showing it to be the softer phase. It is well known in the metallurgical art that fabricability or ductility can be improved if working will convert the softer phase into a continuous phase. After subjecting Alloy A to the above force, the microstructure of the alloy was again examined at 750 magnification. The working of the alloy was found to have caused the hard continuous phase to be broken into small discontinuous fragments. It was observed that the continuous phase in the microstructure was the softer phase, thus indicating an improvement in the ductility of the metal.

## EXAMPLE IV

A 155 gram ingot of the following composition was prepared: 19.2% chromium, 11.2% titanium, and 69.6% niobium, by melting and remelting the metals together 7 times in a water-cooled copper crucible of an arc melting furnace of the type described by Kroll in the "Transactions of the Electrochemical Society" publication referred to above. An atmosphere of helium was used during the heating. When the charge was in the liquid state, the furnace was turned off, and the melt was allowed to cool in the helium atmosphere. When the ingot reached room temperature, it was removed from the water-cooled crucible and machined into a 1/2" cube which has proved highly successful as a high temperature forging die. This alloy has also been made into a high temperature extrusion die.

## EXAMPLE V

75 26.38% by weight of chromium, 14.72% by weight of

titanium, and 68.9% by weight of niobium were charged into the furnace of Example I. The metals were heated under an atmosphere of helium until they were liquid. The melt was then allowed to cool under the helium atmosphere; and after room temperature was reached, the ingot formed in the water-cooled crucible was removed. When this alloy was tested for high temperature oxidation resistance in the manner described for Table I, it showed a 0.65% weight gain over the original as-cast weight of the alloy.

## EXAMPLE VI

Other outstanding alloys within the scope of this invention made according to the procedures of Example I are as follows:

22% titanium, 5% chromium, 71% niobium, 2% cobalt: After 16 hours exposure to air at 1000° C. in accordance with the procedure described in Example I, the gain in weight in the above alloy based on the "as cast" weight of the ingot was 1.4%.

25% titanium, 2.5% chromium, 68% niobium, 2% nickel, 2.5% aluminum: The above alloy after 16 hours exposure to air at 1000° C. in the procedure described in Example I showed a gain in weight of 1.5% based on the "as cast" weight of the ingot prior to exposure.

10.86% titanium, 32.41% chromium, balance niobium: The above alloy after 16 hours exposure to air at 1000° C. in the procedure described in Example I showed a gain in weight of 0.24% based on the "as cast" weight of the ingot prior to exposure.

19% titanium, 3% chromium, 72% niobium, 2% nickel, 4% manganese: When this alloy was exposed to air for 16 hours at 100° C. in the manner described in Example I, it showed a 1.55% gain over the "as cast" weight of the ingot prior to exposure.

12% titanium, 2.5% chromium, 83.5% niobium, 2% nickel

25% titanium, 3% chromium, 70% niobium, 2% aluminum

22% titanium, 4% chromium, 70% niobium, 2% nickel, 2% aluminum

5% titanium, 2% chromium, 90% niobium, 0.5% aluminum, 2.5% zirconium

17.60% titanium, 7.23% chromium, balance niobium, R<sub>c</sub> hardness as cast 47

17.87% titanium, 12.19% chromium, balance niobium, R<sub>c</sub> hardness as cast 45

17.79% titanium, 17.40% chromium, balance niobium, R<sub>c</sub> hardness as cast 46

13.38% titanium, 33.11% chromium, balance niobium, R<sub>c</sub> hardness as cast 47

16.38% titanium, 32.56% chromium, balance niobium, R<sub>c</sub> hardness as cast 58

12.01% titanium, 26.38% chromium, balance niobium, R<sub>c</sub> hardness as cast 55

17.36% titanium, 22.20% chromium, balance niobium, R<sub>c</sub> hardness as cast 48

9% titanium, 10% chromium, balance niobium, R<sub>c</sub> hardness as cast 40

25% titanium, 23% chromium, balance niobium, R<sub>c</sub> hardness as cast 44

10.35% titanium, 33.11% chromium, balance niobium, R<sub>c</sub> hardness as cast 60

25% titanium, 25% chromium, balance niobium, R<sub>c</sub> hardness as cast 50

20% titanium, 28% chromium, balance niobium, R<sub>c</sub> hardness as cast 52

15% titanium, 30% chromium, balance niobium, R<sub>c</sub> hardness as cast 55

5% titanium, 7% chromium, balance niobium, R<sub>c</sub> hardness as cast 47

Although it is preferable to use metals which are of a high purity, a fair amount of variance in purity can be tolerated before product quality suffers appreciably. The alloys of the working examples are made from com-

mercially available metals containing less than 1% incidental impurities. Commercial niobium nearly always contains tantalum (usually in amounts up to 5%) which is hard to detect and very difficult to separate. Therefore, the niobium used to carry out the specific examples no doubt contained tantalum which is reported as niobium rather than as an incidental impurity. In addition to the tantalum which is present in commercial niobium, this invention contemplates the addition of tantalum to the alloy composition in amounts up to 7%. Those skilled in the art are readily aware of the presence of incidental impurities in commercial metals and of the presence of tantalum in commercial niobium, and these facts should be taken into consideration when practicing the invention and construing the claims.

15 The alloys of this invention may be used as a material of construction in any structure which requires a strong, corrosion-resistant metal. Particular stress has been laid upon the use of these alloys in high temperature equipment, such as jet engine parts, nuclear reactor and gas turbine parts because of their outstanding properties. However, it should be emphasized that use of the alloys of this invention is not limited to high temperature conditions or to any piece of equipment described herein.

20 25 Since it is obvious that many changes and modifications can be made in the above-described details without departing from the nature and spirit of the invention, it is to be understood that the invention is not to be limited to said details except as set forth in the appended claims.

30 30 This application is a continuation-in-part of my co-pending application Serial No. 592,705, filed June 4, 1956, now abandoned and also of Serial No. 593,054, filed June 22, 1956, now abandoned. These latter applications are in turn continuations in-part of Serial No. 550,764, filed December 2, 1955, now abandoned.

35 I claim:

1. A high-strength, corrosion-resistant alloy composed of about 5-30% by weight of titanium, about 1-30% by weight of chromium, to which may be added, if desired, up to about 7% by weight of aluminum, up to about 2% by weight of carbon, up to about 2% by weight of cobalt, up to about 7% by weight of iron, up to about 7% by weight of manganese, up to about 2% by weight of nickel, up to about 2% by weight of silicon, up to about 7% by weight of tantalum, up to about 7% by weight of tungsten, up to about 7% by weight of vanadium, up to about 7% by weight of zirconium, the sum total of the added elements Al, C, Co, Fe, Mn, Ni, Si, Ta, W, V and Zr ranging up to about 7% by weight, the balance being niobium in an amount of at least 50% by weight.

40 45 2. The alloy of claim 1 in which the sum total of the added elements Al, C, Co, Fe, Mn, Ni, Si, Ta, W, V and Zr range from about 2-5% by weight.

3. The alloy of claim 1 in which the sum total of the added elements Al, C, Co, Fe, Mn, Ni, Si, Ta, W, V and Zr is about 2% by weight.

45 50 4. A high strength, corrosion-resistant alloy composed of about 5-30% by weight of titanium, about 1-30% by weight of chromium, the balance being essentially niobium in an amount of at least 50% by weight.

5. A high strength, corrosion-resistant alloy composed of about 10-25% by weight of titanium, about 15-30% by weight of chromium, the balance being essentially niobium in an amount of at least 50% by weight.

60 65 6. A high-strength, corrosion-resistant alloy composed of about 10-25% by weight of titanium, about 15-30% by weight of chromium, to which may be added, if desired, up to about 5% by weight of aluminum, up to about 2% by weight of carbon, up to about 2% by weight of cobalt, up to about 5% by weight of iron, up to about 5% by weight of manganese, up to about 2% by weight of nickel, up to about 2% by weight of silicon, up to about 5% by weight of tantalum, up to about 5% by weight of tungsten, up to about 5% by weight of vanadium, up to about 5% by weight of zirconium, the sum

total of the added elements Al, C, Co, Fe, Mn, Ni, Si, Ta, W, V and Zr ranging up to about 5% by weight, the balance being niobium in an amount of at least 50% by weight.

7. A high-strength, corrosion-resistant alloy composed of about 15-25% by weight of titanium, about 20-28% by weight of chromium, to which may be added, if desired, up to about 5% by weight of aluminum, up to about 2% by weight of carbon, up to about 2% by weight of cobalt, up to about 5% by weight of iron, up to about 5% by weight of manganese, up to about 2% by weight of nickel, up to about 2% by weight of silicon, up to about 5% by weight of tantalum, up to about 5% by weight of tungsten, up to about 5% by weight of vanadium, up to about 5% by weight of zirconium, the sum total of the 5 10 15

added elements Al, C, Co, Fe, Mn, Ni, Si, Ta, W, V, and Zr ranging up to about 5% by weight, the balance being niobium in an amount of at least 50% by weight.

References Cited in the file of this patent

UNITED STATES PATENTS

|           |              |               |
|-----------|--------------|---------------|
| 1,588,518 | Brace        | June 15, 1926 |
| 1,742,417 | Schrobsdorff | Jan. 7, 1930  |
| 2,822,268 | Hix          | Feb. 4, 1958  |
| 2,882,146 | Rhodin       | Apr. 14, 1959 |

FOREIGN PATENTS

|         |         |               |
|---------|---------|---------------|
| 718,822 | Germany | Mar. 24, 1942 |
|---------|---------|---------------|